

# United States Patent Office

2,733,975

Patented Feb. 7, 1956

1

2,733,975

## PROCESS OF COATING AND DYEING TEXTILE FIBERS AND RESULTANT ARTICLE

Thomas C. Whitmer, Elizabeth, N. J.

No Drawing. Application July 19, 1950,  
Serial No. 174,777

17 Claims. (Cl. 8—18)

This invention relates to the treatment of textile fibers impregnated with an alkali-copper complex, sericeous material and (in some instances) an alkaline agent. It involves particularly the treatment of such impregnated fibers whereby removal of the alkali-copper complex and of the alkaline agent (if present) is effected and textile fibers are obtained which are impregnated with substantially only sericeous material.

In U. S. Patent 2,417,388 has been described a method of impregnating textile fibers with an aqueous solution in which are dissolved an alkylolamine-copper complex, an alkali metal hydroxide and silk fibers. In my copending application, Ser. No. 761,987, now U. S. Pat. No. 2,565,832, is disclosed a procedure whereby an aqueous solution of an alkylolamine-copper complex, a tetra-alkyl ammonium hydroxide and silk fibers is employed for impregnating textile fibers and in my copending application, Ser. No. 748,674, now U. S. Pat. No. 2,646,372, is described impregnation of textile fibers with aqueous solutions of silk in which a tetra-alkyl ammonium hydroxide serves as both the alkaline substance for forming a copper complex and as the alkaline agent. In my copending application, Ser. No. 101,499, has been disclosed a process whereby an aqueous solution of an alkylolamine-copper complex and sericeous material can be prepared (for impregnation of textile fibers) in which the proportion of alkaline agent (e. g., sodium or potassium hydroxide) is very small. In my copending application, Ser. No. 162,385, now U. S. Pat. No. 2,675,326, is disclosed employment of aqueous solutions in which an alkali metal hydroxide or a tetra-alkyl ammonium hydroxide serves as both the copper complex-forming agent and as the alkaline agent.

In all of the above disclosed methods, the fibers after impregnation with the aqueous solution of copper complex and sericeous material (and while they are still wet or damp and in some instances after the impregnated fibers have been dried) are washed with an aqueous solution of an acidic agent which forms water-soluble salts with the alkali-copper complex and with the alkaline agent (if present). Afterwards, the fibers are washed with water to eliminate substantially all of the salts and acidic agent and to leave them impregnated with substantially only sericeous material.

I have observed that substitution of the aqueous solution of an acidic agent by an aqueous alcoholic solution of an acidic agent, in the above-mentioned procedures, furnishes fibers which contain an increased proportion of sericeous material. Also, I prefer that the aqueous alcoholic solvent for the acidic agent contain a major proportion by volume of the alcohol. To illustrate, two samples of the same cotton cloth are impregnated in the same manner and with substantially the same proportion of the same aqueous solution of alkylolamine-copper complex, sodium hydroxide and sericeous material, and one impregnated sample is washed with an aqueous solution of hydrogen chloride and the other with an aqueous alcoholic (say, 85 per cent isopropyl alcohol) solution of

2

hydrogen chloride. For comparative purposes, the concentration of acidic agent should be the same or substantially so in each solution. Afterwards, each sample is washed well with water and dried. Then it will be found that the cloth washed with aqueous alcoholic acid has gained more proportionally in weight due to treatment than the other cloth, generally will possess a smoother fuller feel, and usually will be dyed to a deeper or darker color when each fabric is dyed in the same manner.

10 In the above-indicated procedure, treatment of the impregnated fibers with aqueous alcoholic acid leads to the formation of alkylolamine hydrochloride, copper (cupric) chloride and sodium chloride. Of these salts, the alkylolamine hydrochloride and copper chloride are soluble in the aqueous alcohol and for the most part will be removed from the fibers during washing with the aqueous alcoholic solution of acid. Sodium chloride, however, has a limited solubility in the alcoholic liquid and it is necessary that the fibers be washed with water so that this salt as well as the acid and any residua of copper and alkylolamine salts be eliminated from the fibers. In other words, I seek to prepare fibers which are impregnated with substantially only sericeous material and are substantially devoid of any salts or acidic agent.

20 I do not mean to limit my invention to the use of inorganic or mineral acids as the above-indicated method can be modified so that organic acids may be employed. For example, cotton cloth impregnated with an aqueous solution of an alkylolamine-copper complex, sericeous material and potassium hydroxide can be washed with an aqueous alcoholic (say, 90 per cent isopropyl) solution of benzoic acid. Afterwards, the cloth is washed with some of the aqueous alcohol to eliminate copper benzoate (which is substantially insoluble in water) as well as unreacted benzoic acid and alkylolamine benzoate. The benzoates of copper and alkylolamine are formed as the result of interaction between benzoic acid and the copper complex. Next, the cloth is washed with water to remove potassium salt. If desired, warm water, e. g., water at a temperature of 50° to 60° C., may be used in this instance in place of water at room temperature as benzoic acid is somewhat more soluble in the warm aqueous liquid and employment of the latter may remove traces of the acid from the treated fibers.

35 Still another modification of my invention involves treatment of fibers impregnated with an aqueous solution of an alkylolamine-copper complex, a tetra-alkyl ammonium hydroxide and sericeous material. In such cases, the impregnated fibers may be washed, for example, with 90 per cent aqueous isopropyl alcohol in which hydrogen chloride is dissolved. Afterwards, the fibers are washed with aqueous alcohol only, since the alkylolamine, tetra-alkyl ammonium and copper salts are soluble in the aqueous alcohol.

50 55 The following examples will furnish additional illustrations of my invention but it will be understood that my invention is not to be limited to them.

Example 1.—To an aqueous solution consisting of 3 g. of copper chloride ( $CuCl_2 \cdot 2H_2O$ ) dissolved in about 20 cc. of water was added triethanolamine in small portions until a dark blue aqueous liquid was obtained in which all the copper compound was dissolved. The liquid then was diluted with water to a volume of 50 cc. In the diluted solution was dissolved sufficient solid sodium hydroxide to react with the amine salt (from interaction of triethanolamine with copper chloride) and to give substantially 1 per cent of the free or uncombined alkali metal hydroxide. During dissolution of the latter compound, the aqueous liquid was cooled externally with water to prevent any appreciable increase in its temperature.

60 65 70 The solution of alkylolamine-copper complex and

alkali metal hydroxide was admixed with 7 g. of silk fibers and the mixture allowed to stand overnight at room temperature. Afterwards, water equal to one-fifth the volume of liquid was added to the mixture and the latter then filtered to remove any undissolved material.

A sample of bleached cotton cloth was impregnated with this filtered solution of sericeous material by immersion in a portion of it for 10 minutes at room temperature. Afterwards, the cloth was allowed to drain at room temperature, washed with aqueous acid (prepared by admixing 1 volume of concentrated aqueous hydrochloric acid with 3 volumes of water), then washed well with water, and dried. Increase in weight of the cloth indicated it contained 1.29 per cent of sericeous material.

Simultaneously, another sample of the same bleached cotton cloth was treated in like manner with this modification: the acidic solution for washing the impregnated cloth was prepared by admixing 1 volume of concentrated aqueous hydrochloric acid with 3 volumes of substantially anhydrous isopropyl alcohol. In this instance, increase in weight of the cellulose material indicated it contained 2.65 per cent of sericeous material.

*Example 2.*—Two grams of copper chloride



were dissolved in 20 cc. of water and to this solution diethanolamine was added slowly and with stirring until a clear blue solution of the copper complex was obtained. Then the aqueous liquid was diluted with water to a volume of 50 cc. Next, sufficient solid potassium hydroxide was dissolved in the solution to react with the amine salt (formed by interaction of diethanolamine with the copper salt) and to furnish substantially 4 per cent of the free or uncombined alkali metal hydroxide. This solution of alkyloamine-copper complex and alkali metal hydroxide was admixed with 6 grams of silk fibers and allowed to stand at room temperature for 1 hour. During this time the mixture was shaken occasionally. Afterwards, water equal to approximately one-fifth the volume of liquid was added to the mixture and the latter then filtered to eliminate undissolved material.

A sample of unbleached cotton cloth was impregnated with some of this filtered solution by immersion therein for 30 minutes at room temperature. The sample then was allowed to drain at room temperature and afterwards was washed twice with aqueous acid prepared by admixing 2 volumes of glacial acetic acid with 38 volumes of water. Next, the fabric was washed with water and dried. Increase in weight indicated it contained 1.68 per cent of sericeous material.

Simultaneously, another sample of the same unbleached cotton cloth was treated in like manner with this modification: the acidic solution for washing the impregnated textile material was prepared by admixing 2 volumes of glacial acetic acid, 2 volumes of water and 36 volumes of substantially anhydrous n-propyl alcohol. In this instance, increase in weight of the sample indicated it contained 4.23 per cent of impregnating material.

*Example 3.*—Copper hydroxide was admixed with water and to the mixture was added slowly diethanolamine until the copper compound dissolved and a blue-colored solution was obtained. The latter then was diluted with water to give an aqueous solution in which the concentration of copper was equivalent to 2.66 g. of copper hydroxide per 100 cc. of liquid. In this solution was dissolved sufficient potassium hydroxide to furnish substantially 4 per cent of the alkali metal hydroxide. Silk fibers were admixed with this solution of copper complex and alkali metal hydroxide (maintained at room temperature) over a period of 1 hour until an excess of the fibers had been added. The liquid then was separated from undissolved fibers by filtration.

Two samples of unbleached cotton cloth were im-

regnated separately with some of the filtered solution. In each instance, the fabric was worked in the liquid at room temperature for 15 minutes, then removed and allowed to drain at room temperature. One of the impregnated fabrics was washed twice with an acid solution prepared by admixing 5 volumes of 85 per cent aqueous lactic acid with 35 volumes of water. Afterwards, the fabric was washed well with water and dried. Increase in weight of this sample indicated it contained 0.75 per cent of impregnating material.

The other impregnated fabric was washed with an acidic solution prepared by admixing 5 volumes of 85 per cent aqueous lactic acid, 4 volumes of water and 31 volumes of glycerine. In this instance, the acidic solution was rather viscous and consequently it was taken up very slowly by the impregnated cloth. Also, the alkaline bodies and copper complex (present in the impregnated cloth) reacted slowly with the acid. It was necessary in this case that the fabric remain immersed in the aqueous alcoholic acid for approximately 16 hours at room temperature. And during that time the acidic solution was stirred occasionally to insure, as far as possible, that the aqueous glycerine solution in contact with the cloth was always acidic in character. Afterwards, the treated cloth was washed well with water and dried. Increase in weight of this sample indicated that it contained 7.79 per cent of impregnating material.

The two treated samples and also one of the original unbleached cotton material were dyed separately and in each instance the dye bath consisted of 100 parts of water per 1 part of cloth and 5 per cent (on weight of sample) of a basic dye (Malachite Green). The samples were immersed in their respective baths at room temperature, and after 15 minutes the temperature of the baths was increased to 65° C. over a period of 30 minutes, then kept at 65° to 70° C. for 30 minutes, and afterwards the baths were allowed to cool to room temperature. Then the fabrics were removed, rinsed well with cold water, and dried. The untreated cloth was a light bluish green in color; the sample which during treatment had been washed with aqueous acid was slightly darker in color and had less of the bluish cast; the sample which during treatment had been washed with the aqueous glycerine solution of acid was much darker in color than either of the other two fabrics, was predominately green in color with little of the bluish cast, and possessed a firmer and smoother feel than either of the other samples.

*Example 4.*—To 3 g. of copper chloride



dissolved in 50 cc. of water was added triethanolamine slowly and in small amounts until a deep blue aqueous solution of the copper complex was obtained. The liquid then was diluted with water to a volume of 100 cc. In this solution was dissolved sufficient sodium hydroxide to react with the alkyloamine salt (from interaction of alkyloamine and copper salt) and to give substantially 3 per cent of the alkali metal hydroxide. Silk fibers were admixed with the liquid (keeping the quantity of fibers in excess of that which dissolved) and the mixture allowed to stand with occasional stirring for 2 hours at room temperature. Afterwards, the liquid was filtered from undissolved fibers.

Two samples of unbleached cotton cloth were impregnated separately at room temperature with the filtered solution. One of the impregnated samples then was washed with 8 per cent aqueous sulfuric acid in which was dissolved 2 per cent of sodium sulfate, afterwards washed with water, and dried. Increase in weight of this fabric indicated it contained 3.36 per cent of sericeous material.

The other sample of impregnated cloth was washed with an 8 per cent solution of benzoic acid in a solvent consisting of 95 volumes of n-propyl alcohol and 5 volumes of water. In this instance, three successive portions of

the acidic solution were used. Afterwards, the cloth was washed with some of the aqueous alcholic solvent, then with water, and dried. Increase in weight of this fabric indicated it contained 5.16 per cent of sericeous material.

As the function of the acid is to react with the copper complex and with the alkaline agent and thereby precipitate sericeous material in or on the fibers, the quantity of acid in solution as well as its concentration should be such that more than sufficient acid for such reactions is present and the liquid in direct contact with the fibers should be appreciably acidic at all times. Because of the small solubility of benzoic acid in water, it seemed inadvisable in this instance to compare the effect of this acid in aqueous solution with that of the acid in aqueous alcohol. If aqueous benzoic acid had been employed, then a large proportion of alkylolamine-copper complex and alkali metal hydroxide (and consequently of sericeous material) would have been washed out of the impregnated fibers prior to reacting with the acid due to the large volume of water needed to dissolve the required quantity of acid. For these reasons, an acid more soluble in water, namely, sulfuric acid, was used when water only was the solvent. Also, a small proportion of alkali metal salt was dissolved in the aqueous acid to aid in precipitation of sericeous material. Employment of an aqueous acid containing a small proportion of a dissolved alkali metal salt in the treatment of textile fibers impregnated with an alkylolamine-copper complex and sericeous material has been described in my copending application Ser. No. 101,499.

*Example 5.*—To 5 g. of copper chloride



dissolved in a small quantity of water was added 2-amino-2-methyl-propanediol-1,3 in small portions and with stirring until all of the copper compound was changed into the alkylolamine-copper-complex and a deep blue colored solution was obtained. The latter then was diluted with water to a volume of 100 cc. Next, sufficient potassium hydroxide was dissolved in the aqueous solution to react with the alkylolamine salt (resulting from interaction of alkylolamine with copper compound) and to give substantially 3 per cent of the uncombined alkali metal hydroxide. Silk fibers, in an amount greater than that which would dissolve, were admixed with the aqueous solution and the mixture allowed to stand for 2 hours at room temperature. Afterwards, undissolved fibers were separated by filtration.

Two samples of unbleached cotton cloth were impregnated with some of the filtered solution by immersion therein at room temperature. The two samples were allowed to drain and to remain exposed to the atmosphere overnight. One of these samples was washed with 10 per cent aqueous hydrochloric acid, then with water, and dried. Increase in weight of this sample indicated it contained 4.43 per cent of sericeous material.

The other fabric was immersed in a 10 per cent solution of salicylic acid in a solvent consisting of 95 volumes of propylene glycol and 5 volumes of water. The cloth was permitted to remain immersed in this acidic liquid at room temperature for about 18 hours (overnight). Afterwards, the sample was removed, washed well with cold water, then washed with warm water (temperature, 50° to 55° C.), and dried. Increase in weight of this fabric indicated it contained 9.02 per cent sericeous material.

The reasons for comparing washing of one sample with aqueous hydrochloric acid with washing of the other sample with salicylic acid in an aqueous alcholic solution are similar to those given under Example 4 for comparing the effect of aqueous sulfuric acid with that of benzoic acid in an aqueous alcholic solution.

*Example 6.*—To a mixture of 2.5 g. of copper hydroxide and 100 cc. of 70 per cent aqueous ter.-butyl alcohol was added 2-amino-2-methyl-propanediol-1,3 in small portions

until all of the copper compound dissolved and a deep blue colored solution was obtained. In this solution was dissolved sufficient solid sodium hydroxide to give substantially 2.5 per cent of the alkali metal hydroxide.

This solution was admixed with a relatively large quantity of silk fibers and the mixture allowed to stand at room temperature, with occasional stirring, until the supernatant liquid possessed only a very light blue color. The alcholic liquid then was separated from the treated fibers and the latter were washed twice with large portions of 70 per cent aqueous ter.-butyl alcohol. Each time, the alcholic liquid was drained as completely as possible from the fibers and the latter were pressed to eliminate as well as possible whatever liquid was retained by them. The treated and washed fibers were admixed with 100 cc. of water and the mixture allowed to stand overnight. Filtration of the liquid then removed undissolved fibers. This method of preparing aqueous solutions of sericeous material is described in my copending application Ser. No. 101,499.

Two bleached cotton cloth samples were impregnated with some of the filtered aqueous solution of sericeous material, and then allowed to drain and to dry at room temperature. One sample was washed with aqueous 10 per cent sulfuric acid, then with water, and dried. Increase in weight of this sample indicated it contained 5.52 per cent of sericeous material.

The other sample was washed with 80 per cent aqueous isopropyl alcohol in which was dissolved substantially 10 per cent by weight of concentrated sulfuric acid. Afterwards, the sample of cloth was washed with water and dried. Increase in weight of this fabric indicated it contained 8.48 per cent of sericeous material.

*Example 7.*—An aqueous solution of sericeous material was prepared in the following manner: 14 volumes of water were mixed with 6 volumes of glycerine and then lithium hydroxide was dissolved in the aqueous alcholic liquid in the proportion of 1.2 g. to 20 cc. of liquid. Afterwards, the alkaline solution was saturated with copper hydroxide ( $\text{Cu}(\text{OH})_2$ ) by admixing the latter with the alkaline solution in small portions and stirring the mixture. When an excess of the copper hydroxide had been added, the mixture of liquid and solid was allowed to stand overnight at room temperature. Then the resulting blue solution was separated from undissolved copper compound by filtration.

Silk fibers were admixed with the solution of copper compound in the proportion of 5 g. of fibers to 20 cc. of liquid. After the mixture had stood, with occasional stirring, at room temperature for 1 hour, the resulting pasty mass was diluted with a volume of water equal to 1.5 times that of the initial solution of copper compound. The diluted mixture was permitted to stand for a few minutes at room temperature and then was filtered. Substantially all of the silk fibers had dissolved.

Two samples of the same bleached linen cloth were impregnated with some of the filtered solution. After the samples had drained, one of them was washed with dilute aqueous hydrochloric acid, then with water, and dried. Increase in weight of this sample indicated it contained 0.67 per cent of impregnating material.

The other impregnated sample, after draining, was washed with three separate portions of aqueous alcholic acid made by admixing 15 volumes of concentrated hydrochloric acid, 15 volumes of water and 70 volumes of substantially anhydrous isopropyl alcohol. Next, this fabric was washed well with water, and dried. Increase in its weight indicated it contained 1.53 per cent of impregnating material.

*Example 8.*—An aqueous solution containing substantially 20 per cent of tetraethanol ammonium hydroxide was admixed with copper hydroxide ( $\text{Cu}(\text{OH})_2$ ) and the admixture allowed to stand at room temperature, with occasional stirring, until no more of the copper compound

appeared to dissolve. The blue colored solution then was separated from undissolved copper hydroxide.

Silk fibers were admixed with the aqueous solution of copper complex and allowed to stand, with occasional stirring, for 18 hours at room temperature. Afterwards, undissolved fibers were eliminated by filtration of the mixture.

Two samples of unbleached cotton cloth were saturated with some of the filtered aqueous sericeous solution by working therein at room temperature. Then both samples were permitted to drain and to dry by exposure to the atmosphere. One sample was washed with dilute aqueous sulfuric acid, then with water, and dried. Increase in weight of this cloth indicated it contained 1.4 per cent of impregnating material. This procedure, includes the preparation of aqueous solutions containing substantially only a tetra-alkylol ammonium hydroxide-copper complex and silk and the application of such solutions to the treatment of cellulose fibers, is described in my copending application Serial No. 221,323.

The other sample was washed three successive times with portions of an acidic solution prepared by admixing 5 volumes of concentrated sulfuric acid, 15 volumes of water, and 80 volumes of substantially anhydrous isopropyl alcohol. Next, it was washed with water, and dried. Increase in weight of this fabric indicated it contained 8.03 per cent of impregnating material.

As previously mentioned in this specification, the alcohols which I prefer are water-soluble, acyclic, saturated, normally-liquid compounds. They may be either monohydroxy or polyhydroxy. The alcohols should be sufficiently soluble in water or should be capable of dissolving sufficient water so that the resulting aqueous alcoholic liquid will not contain less than about 60 per cent by volume of the alcohol. Aqueous alcoholic liquids containing a greater proportion by volume of the alcohol, say, 80 or 90 per cent, also are suitable. If necessary or desirable, the alcoholic liquid may have only a very small proportion of water, say, 0.5 to 1 per cent by volume, and may even be substantially anhydrous. Mixtures of alcohols are permissible, provided the total alcoholic content of the aqueous liquid is not less than about 60 per cent.

By the term saturated I mean that the alcohols do not contain any unsaturated (e.g., olefinic or acetylenic) linkages in their molecular structures. By the term normally liquid I mean that the alcohols are liquids at room temperature or thereabouts. Examples of such alcohols are ethyl, isopropyl or ter.-butyl alcohol, propylene or trimethylene glycol, and glycerine. Alcohols which are solids at temperatures appreciably higher than room or atmospheric temperature, e.g., mannitol, are not included in this invention.

I have illustrated my procedure with fibers which have been impregnated with aqueous solutions containing, in addition to dissolved silk fibers, a complex compound of copper. Examples of such copper complexes are an alkylolamine-copper complex, an alkali metal hydroxide-copper complex, a tetra-alkylol ammonium hydroxide-copper complex and a tetra-alkyl ammonium hydroxide-copper complex. The alkylolamines suitable for my purpose can be either a primary, secondary or tertiary amine or they can be either monohydroxy or polyhydroxy compounds. The tetra-alkylol ammonium hydroxides and the tetra-alkyl ammonium hydroxides may be compounds in which all four groups (alkylol or alkyl) are the same or in which two or more of these groups differ from the others. My invention is applicable also to the treatment of cellulose fibers impregnated with aqueous solutions containing, in addition to dissolved silk fibers, other alkali copper complexes, e.g., those formed by interaction of ammonia or of primary, secondary or tertiary amines with copper hydroxide. Since all these complexes either contain copper and an alkaline compound or are the result of interaction of a copper compound with an alkaline compound to furnish a water-soluble substance, I include all

such complexes under the general term of alkali-copper complex. It should be noted that the alkaline compounds may be inorganic (e.g., ammonia or sodium hydroxide) or organic (e.g., ethylamine or diethanolamine) in character.

5 The impregnated cellulose fibers may be treated according to this invention while they are still wet with the aqueous solution containing the copper-complex and dissolved silk fibers. Or, the impregnated fibers may be partially or substantially dry prior to treatment. Preferably the drying operation is effected at room or atmospheric temperature or thereabouts and thereby avoid any harmful action on the cellulose fibers or on the sericeous material impregnated therein.

10 The acidic agents suitable for my purpose can be either inorganic or organic (carboxylic) compounds. Illustrations of inorganic acids are hydrochloric, hydrobromic or sulfuric acid. Examples of carboxylic acids are acetic or benzoic acid. Substituted carboxylic acids such as lactic acid, salicylic acid, chloracetic acid and bromobenzoic acid may be employed also. In some instances the hydroxy-substituted acids, such as lactic or salicylic acid, are particularly applicable since they furnish copper salts which exhibit appreciable solubilities in water and in alcohol. Whatever acidic agents are employed, they should meet the following conditions: (1) should not react in any undesirable manner with the aqueous alcoholic liquid, (2) should not be present in sufficient concentration in the aqueous alcoholic solution so as to exert any deleterious action of the cellulose fibers or on the sericeous material impregnated therein, and (3) should furnish salts, on reaction with the alkaline agent and copper complex, which are appreciably soluble in water or in the aqueous alcoholic liquid or in both.

15 25 When cellulose fibers impregnated with an alkali-copper complex and sericeous material are washed with the aqueous alcoholic solution of acidic agent, the latter should be present in sufficient quantity to react with all the alkaline agent (if present) and all of the copper complex. This step of washing the impregnated fibers requires somewhat more time than if an aqueous solution of the acidic agent is employed. In the case of polyhydroxy alcohols, such as propylene glycol or glycerine, which furnish (when employed in accordance with the method of this invention) rather viscous solutions of acidic agent, immersion of the impregnated fibers for several hours in the acidic liquid is often required to effect substantially complete conversion of the copper complex into the corresponding copper salt. Moreover, I do not wish to be limited to one washing of the fibers with the aqueous alcoholic solution of acidic agent. If necessary, fibers impregnated with alkali copper complex and sericeous material may be washed two or more successive times and each operation involves employment of an unused portion of the acidic solution.

20 25 30 After the fibres are treated with the acidic solution, they are washed with the aqueous alcoholic solvent, or with water, or successively with the aqueous alcoholic solvent and with water. The solvent or solvents used in this operation will depend upon such factors as the alkali-copper complex and the aqueous alcohol and the acidic agent dissolved therein. For example, if cellulose fibers are impregnated with an aqueous solution containing alkylolamine-copper complex, alkali metal hydroxide and dissolved silk fibers and are washed with an acidic solution consisting of sulfuric acid dissolved in aqueous isopropyl alcohol, then the acid wash should be followed by one with water so as to eliminate any alkali metal sulfate and copper sulfate which may not be removed by the aqueous alcoholic liquid. Or, if the same impregnated fibers be washed with an acidic solution of benzoic acid in aqueous isopropyl alcohol, then it is essential that the fibers be washed afterwards with aqueous alcohol, to eliminate copper benzoate, prior to the water wash. In any event, the liquids employed subsequent to treatment of the fibers with the solution of acidic

agent should remove substantially all salts, acidic agent and alcohol (if not readily evaporated at room temperature or thereabout) from the fibers and leave them impregnated with substantially only sericeous material.

Although I have illustrated the process of this invention by its application to the treatment of cellulose fibers, I do not wish to be limited to the treatment of such fibers. Some of the aqueous solutions containing dissolved sericeous material (as a copper-containing complex) and a small proportion of alkaline bodies, as for example those 10 solutions described in my copending application Ser. No. 101,499, can be employed for impregnation of animal fibers (such as wool or silk) with sericeous material. Animal fibers impregnated with such aqueous solutions or copper-silk complexes and alkaline bodies may be 15 treated according to the method of this invention.

What I claim is:

1. The process for treating textile fibers impregnated with a water-soluble alkali-copper complex selected from the group consisting of alkylamine containing no alkylol groups-, alkylolamine-, tetra-alkylol ammonium hydroxide-, and alkali-metal hydroxide-copper complexes, and sericeous material which comprises washing said fibers with aqueous alcohol containing a dissolved acidic agent, and then washing the fibers with aqueous alcohol, said aqueous alcohol consisting of an admixture of a saturated acyclic normally-liquid water-soluble alcohol and water and containing at least about 60 per cent by volume of said alcohol, and said acidic agent forming salts with said copper complex which are soluble in said aqueous alcohol which acidic agent does not interfere in any undesirable way with the aqueous alcohol and is present in amount insufficient to exert any deleterious action on the fibers and sericeous material.

2. The process according to claim 1 in which the water-soluble alcohol is a monohydroxy alcohol.

3. The process according to claim 1 in which the water-soluble alcohol is a dihydroxy alcohol.

4. The process according to claim 1 in which the water-soluble alcohol is a trihydroxy alcohol.

5. The process for treating textile fibers impregnated with a water-soluble alkali-copper complex selected from the group consisting of alkylamine containing no alkylol groups-, alkylolamine-, tetra-alkylol ammonium hydroxide-, and alkali-metal hydroxide-copper complexes, and sericeous material which comprises washing said fibers with aqueous alcohol containing a dissolved acidic agent, then washing the fibers with aqueous alcohol, and afterwards washing the fibers with water, said aqueous alcohol consisting of an admixture of a saturated acyclic normally-liquid water-soluble alcohol and water and containing at least about 60 per cent by volume of said alcohol, and said acidic agent forming salts with said copper complex which are soluble in a solvent selected from the

group consisting of water and said aqueous alcohol which acidic agent does not interfere in any undesirable way with the aqueous alcohol and is present in amount insufficient to exert any deleterious action on the fibers and sericeous material.

5. The process according to claim 5 in which the acidic agent is a mineral acid.

6. The process according to claim 5 in which the acidic agent is a monocarboxylic acid.

7. The process according to claim 5 in which the acidic agent is a monohydroxy monocarboxylic acid.

8. The process according to claim 5 in which the acidic agent is a monohydroxy monocarboxylic acid.

9. In a process of treating textile fibers impregnated with a water-soluble alkali-copper complex selected from the group consisting of alkylamine containing no alkylol groups-, alkylolamine-, tetra-alkylol ammonium hydroxide-, and alkali metal hydroxide-copper complexes, and sericeous material, which comprises washing said fibers with aqueous alcohol containing a dissolved acidic agent, said aqueous alcohol consisting of an admixture of a saturated acyclic normally-liquid-water-soluble alcohol and water and containing at least about 60% by volume of said alcohol, and said acidic agent forming salts with said copper complex which are soluble in said aqueous alcohol which acidic agent does not interfere in any undesirable way with the aqueous alcohol and is present in amount insufficient to exert any deleterious action on the fibers and sericeous material.

10. The process according to claim 9 in which the water soluble alcohol is a monohydroxy alcohol.

11. The process according to claim 9 in which the water soluble alcohol is a dihydroxy alcohol.

12. The process according to claim 9 in which the water soluble alcohol is a trihydroxy alcohol.

13. The process according to claim 1 which includes the further step of dyeing the washed textile fibers.

14. The process according to claim 5 which includes the further step of dyeing the washed textile fibers.

15. The process according to claim 9 which includes the further step of dyeing the impregnated textile fibers.

40 16. Textile fibers impregnated with substantially only sericeous material, resulting from the method of claim 1.

17. Dyed textile fibers, the fibers being impregnated with substantially only sericeous material, resulting from the method of claim 1.

#### References Cited in the file of this patent

#### UNITED STATES PATENTS

|           |         |               |
|-----------|---------|---------------|
| 1,936,753 | Dreyfus | Nov. 28, 1933 |
| 1,955,221 | Borner  | Apr. 17, 1934 |
| 2,417,388 | Whitner | Mar. 11, 1947 |
| 2,417,389 | Whitner | Mar. 11, 1947 |
| 2,446,682 | Whitner | Aug. 10, 1948 |
| 2,565,832 | Whitner | Aug. 28, 1951 |